

Oct. 10, 1933.

H. SCOTT

1,929,655

OXIDATION RESISTANT BIMETAL

Filed July 17, 1931



WITNESSES:

*Peter J. McManon*  
*N. M. McManon*

INVENTOR

Howard Scott

BY  
*M. R. Coley*  
ATTORNEY

Patented Oct. 10, 1933

1,929,655

# UNITED STATES PATENT OFFICE

1,929,655

## OXIDATION RESISTANT BIMETAL

Howard Scott, Wilkinsburg, Pa., assignor to Westinghouse Electric & Manufacturing Company, a corporation of Pennsylvania

Application July 17, 1931. Serial No. 551,441

3 Claims. (Cl. 297—15)

My invention relates to thermally actuatable devices and particularly to bimetal thermostatic elements.

An object of my invention is to provide a bimetal element that shall be made of material capable of resisting oxidation, able to withstand subjection to relatively high temperatures, be able to withstand repeated cycles of heating and cooling without loss of strength and have a linear deflection in accordance with temperature changes.

In practicing my invention, I provide a bimetal element, both components of which include an appreciable, but not major, percentage of chromium, relatively small percentages each of silicon, manganese and carbon, the remainder being iron. The high-expansion component has not over 9% of chromium and need not contain over 25% of nickel, although a higher nickel content is permissible, while the low-expansion component may have a chromium content varying 8% to 23% and traces only of nickel.

The single figure of the drawing is a view, in section, of a bimetal bar embodying my invention.

Referring to the drawing, I have indicated a bimetal bar as including a high-expansion component 11 and a low-expansion component 12, each of a composition to be hereinafter set forth, the two components or elements being suitably secured together, as by welding, in a manner now well known in the art. While I have indicated a specific form of bimetal element, such as a bar, my invention is not limited thereto but resides more particularly in the compositions of the two components of the device.

One of the relatively difficult applications of a bimetal thermostat is that of being utilized to signal or indicate the failure of a pilot flame, and, in an application of this kind, it is necessary that the bimetal element shall have a relatively high resistance to oxidation. A further very desirable characteristic is that the bimetal element shall have sufficient mechanical strength to be able to withstand subjection to temperatures of 500° C. or over without loss of mechanical strength, even after having been subjected to a relatively large number of cycles of heating and cooling. That is, it is highly desirable that the deflection be always the same for a given temperature variation, in order to avoid recalibration or resetting of the adjustable element of the device. A relatively large deflection is not of as great importance in an application of this kind as are the other characteristics hereinbefore set forth. Another desirable characteristic is that the deflection of a bimetal bar, when one of its ends is fixed and the other is free to move in response to temperature variations, shall be linear, that is, it shall be the same

per unit change of temperature at any part of its working range of temperature.

I have found that such characteristics are inherent in a bimetal element including two chromium steels, one of which contains sufficient nickel, together with manganese and carbon, to render it substantially non-magnetic at atmospheric temperatures. This non-magnetic alloy has a high expansivity, nearly that of brass. My other chromium steel contains little or no nickel, and is magnetic. Usually, it contains a larger percentage of chromium than the non-magnetic component, say 13 percent chromium, and it has a lower expansion than ordinary steel. Preferably, both elements are high-chromium steels, that is, steels having more than 2 or 3 percent of chromium, so as to obtain the desired corrosion-resistant, heat-resistant characteristic.

Thus, I have found that the high-expansion component 11 may have a chromium content varying between 2% and 9%, a nickel content varying between 18% and 25%, or possibly more, a silicon content varying between .1% and 2%, a manganese content varying between .4% and 2%, a carbon content of less than .5%, the remainder being iron and traces of other elements which may be considered impurities. By nickel, I mean to include commercial nickel, which usually has a small quantity of cobalt mixed in with it.

The low-expansion component 12 may have a chromium content varying between 8% and 23%, or possibly more, a nickel content so small that it may be considered an impurity, that is, below 1%, a silicon content of the order of .1% to 3% or even more, a manganese content of the order of .2% to 1%, a carbon content less than .5%, the remainder being iron and traces of other elements. These proportions for the two elements 11 and 12 are preferred values, and are given mainly to indicate certain alloys which are possible to be used.

A suitable bimetal element may be chosen from the following compositions:

| Alloy symbol | Composition |      |      |      |      | 110 |
|--------------|-------------|------|------|------|------|-----|
|              | % Cr        | % Ni | % Si | % Mn | % C  |     |
| I            | 7.8         | 19.5 | 0.78 | 0.61 | 0.47 |     |
| II           | 7.2         | 21.9 | 1.87 | 0.82 | 0.47 |     |
| A            | 13.0        | 0.2  | 0.3  | 0.5  | 0.1  |     |
| B            | 20.3        | 0.6  | 2.8  | 0.85 | 0.44 | 115 |
| C            | 8.4         | 0.1  | 3.2  | 0.54 | 0.45 |     |

The alloys identified by I and II are high-expansion steels and those identified by A, B and C are comparatively low-expansion steels.

Their expansion is given approximately in the following table:

| 5  | Alloy symbol | Mean expansivity from 0° C. to:         |                                         |                                         |
|----|--------------|-----------------------------------------|-----------------------------------------|-----------------------------------------|
|    |              | 100° C.                                 | 300° C.                                 | 500° C.                                 |
| 10 | I            | $17.8 \times 10^{-6}/^{\circ}\text{C.}$ | $18.5 \times 10^{-6}/^{\circ}\text{C.}$ | $19.2 \times 10^{-6}/^{\circ}\text{C.}$ |
|    | II           | 17.4                                    | 18.0                                    | 18.6                                    |
|    | A            | 9.9                                     | 10.7                                    | 11.5                                    |
|    | B            | 10.5                                    | 11.3                                    | 12.1                                    |
|    | C            | 11.2                                    | 11.9                                    | 12.6                                    |
|    | Difference   | 7.9                                     | 7.8                                     | 7.7                                     |
|    | I minus A    |                                         |                                         |                                         |

15 The sensitivity of the bimetal element is proportional to the difference in expansivity of the components. From the difference between the best tabulated values it is apparent that the deflection of such a bimetal element is nearly as high as that of monel and 42 percent nickel steel and that it is practically linear.

20 I have found that it is relatively easy to fabricate my bimetal elements by suitably welding together relatively heavy ingots of the two alloys at a relatively high temperature and then rolling the same to the desired thickness of the bimetal bar, sheet or disc. Samples of such bimetal elements have withstood the oxidizing effect of high temperatures on the order of 500° C. and over, and the deflection is a linear one, that is, it varies in accordance with the variation of the temperature, and I have found that the deflection per unit change of temperature is substantially the same over a temperature range of 100° C. and 500° C.

25 35 The bimetal element embodying my invention thus provides a thermally actuable metallic thermometer structure which is highly resistant to oxidation, which will stand subjection to a large number of cycles of operation without loss of mechanical strength, which will stand relatively high temperatures without loss of mechanical strength, and the deflection of which is substantially a linear function of temperature change.

40 45 As various modifications may be made in the device embodying my invention without departing from the spirit and scope thereof, I desire that only such limitations shall be placed thereon as are imposed by the prior art.

I claim as my invention:

1. A bimetal element having a high-expansion component of the following composition; approximately 5.7% chromium, approximately 22% nickel, approximately .2% silicon, approximately seven-tenths per cent of manganese, approximately forty-seven hundredths per cent of carbon and substantially all of the remainder iron, and having a low-expansion component of the following composition; approximately 17% chromium, approximately one per cent each of silicon and manganese, from one-tenth per cent to forty-five hundredths per cent of carbon, a trace of nickel and substantially all of the remainder iron.

2. A bimetal element including two chromium-steel alloys of different temperatures expansivities, the high-expansion component having the following composition:

|           |                  |     |
|-----------|------------------|-----|
| Chromium  | Per cent         | 95  |
| Nickel    | 2. to 9.         |     |
| Silicon   | 18. to 25.       |     |
| Manganese | .1 to 2.         |     |
| Carbon    | .4 to 2.         |     |
| Iron      | approximately 47 | 100 |
|           | remainder        |     |

and the low-expansion component having the following composition:

|           |           |     |
|-----------|-----------|-----|
| Chromium  | Per cent  | 105 |
| Nickel    | traces    |     |
| Silicon   | .1 to 3.2 |     |
| Manganese | .2 to 1.  |     |
| Carbon    | .1 to .45 |     |
| Iron      | remainder | 110 |

3. A bimetal element having a high expansion component of the following composition; between 7.2% and 7.8% chromium, between 19.5% and 21.9% nickel, between .78% and 1.87% silicon, between .61% and .82% manganese, approximately .47% carbon, the remainder being principally iron, and a low expansion component of the following composition; between 8.4% and 20.3% chromium, between .3% and 3.2% silicon, between 1.1% and .6% nickel, between .5% and .85% manganese, between .1% and .45% carbon, the remainder being principally iron.

HOWARD SCOTT. 125

55

130

60

135

65

140

70

145

75

150